

1

3,052,632

**HIGH TEMPERATURE GREASE COMPOSITIONS**  
 Donald E. Loeffler, Walnut Creek, Calif., assignor to  
 Shell Oil Company, a corporation of Delaware  
 No Drawing. Filed Feb. 11, 1959, Ser. No. 792,463  
 5 Claims. (Cl. 252—51.5)

This invention relates to lubricating grease compositions. More especially it relates to improved grease compositions especially useful at elevated operating temperatures.

As lubricants are required to perform at higher and higher temperatures because of increased speeds of engines and machines, the advent of jet propulsion and atomic energy as sources of power, etc., it has become increasingly difficult to provide greases fulfilling the requirements of such lubricants. In attempting to provide suitable greases, the art has progressed from the use of petroleum lubricant vehicles thickened with metal soaps of long chain fatty acids to more thermally stable synthetic lubricating oils such as the aliphatic diesters, silicone polymers, etc. thickened with such soaps or inorganic materials, such as silica gels or clays. The progress of thickener research has not in general kept pace with the development of lubricant vehicles. At operating temperatures as high as 400—450° F., there are few greases available which will retain their consistency and lubricity for any substantial period of time.

One of the prominent advances in the art of high temperature grease lubrication has comprised the provision of greases gelled with dyes or pigments, namely, indogen compounds, phthalocyanine compounds, anthraquinones, azines, and especially indanthrene compounds. The art of preparing greases from these particular classes of materials has not been developed. Consequently, the greases comprising such dyes normally require excessive amounts of the gelling agent to produce the grease structure.

It is an object of the present invention to provide improved grease compositions. It is another object of the present invention to provide grease compositions especially useful at high operating temperatures. It is a particular object of the present invention to provide dye gelled greases having a reduced dye requirement for a given grease consistency. It is a special object of the present invention to reduce the high cost of dye gelled greases. Other objects will become apparent during the following description of the invention.

Now, in accordance with the present invention, it has been found that the consistency of greases gelled with indanthrene compounds may be materially increased by the incorporation of 2.5—20% by weight, based on the grease, of diaryl amines having the general configuration



wherein each Ar is an aromatic hydrocarbon radical of the group consisting of phenyl naphthyl, alkylated phenyl and alkylated naphthyl radicals.

In further accordance with the invention, an additional unexpected advantage is obtained in the prolonged high temperature bearing life of the grease compositions. This is especially surprising in view of the fact that the diaryl amines above are less thermally stable than the indanthrene dyes.

Another unexplainable feature of the invention is that the use of diaryl amines to increase consistency appears to be restricted to greases gelled with indanthrene compounds, since addition of the same amines to greases gelled with other high temperature gelling agents either had no effect on consistency or actually softened the grease.

2

The chief benefit derived from the present invention comprises a drastic reduction in the cost of the subject greases. This is material since the principal gelling agent, namely, the dyes are extremely expensive materials while the amines are far less costly. For example, the indanthrene dyes at the present time cost in the order of \$11.00 a pound while the amines are currently priced at 60—70 cents a pound. Consequently, any reduction in the dye content of the grease by a corresponding addition of the 10 amine results in an approximate twenty-fold saving in grease thickener cost. However, not only is this cost reduction a principal factor but also the unexpected improvement in bearing life caused by the presence of the large quantities of amines present constitutes an impressive improvement in lubricating greases of this particular class.

While the proportion of amine normally utilized for increasing the consistency of the subject grease compositions is between 2.5 and about 20% by weight thereof, 20 another measure of the suitable proportions may be expressed in terms of equivalents of dye per hundred grams of grease. The maximum effect is obtained if between about 0.02 and 0.1 equivalents of amine per hundred grams of grease is utilized, although substantial increases 25 in consistency and in bearing life are obtained when the proportion of amine is between about 0.005 and 0.2 equivalents per one hundred grams of grease.

Suitable diaryl amines include the following:

30 Phenyl-alpha-naphthylamine  
 Phenyl-beta-naphthylamine  
 Diphenylamine  
 Di(alpha-naphthyl)amine  
 Di(beta-naphthyl)amine  
 35 (Alpha-naphthyl)(beta-naphthyl)amine  
 Di(tert-butylphenyl)amine  
 (Sec-amylphenyl)phenylamine  
 (Methylphenyl)naphthylamine

40 Preferably, any alkyl substituents on the aryl nuclei have 1—10 carbon atoms each.

The amines are preferably incorporated by homogenizing them with the finished grease containing the principal thickening agent and the lubricating oil. However, the 45 amines may be incorporated with the thickener at the time the grease is originally prepared or may be dispersed in lubricating oil prior to addition of the principal thickening component.

The most effective dye for use in high temperature 50 greases has been found to be the parent compound of the series, namely, indanthrene itself, but other indanthrene compounds may be employed. It is best to utilize the indanthrene compounds in their non-metallic form, that is, 55 without neutralization of the carbonyl groups in said compounds with such ions as sodium or potassium, calcium, etc. While it is possible to employ the partially or fully neutralized indanthrene compounds as grease thickening agents, greases having maximum lubricating life at elevated temperatures are those in which the carbonyl groups are free of any metallic substituents. Typical indanthrene compounds suitable for the present purpose include the following:

65 Indanthrene  
 Flavanthrone  
 Pyranthrone  
 Violanthrone  
 3,3'-dichloroindanthrene  
 70 3-chloroindanthrene

The indanthrene dyes, which are used as the gelling

agents in the subject greases, contain two units of the following essential typical grouping per molecule:



The tricyclic radical, it will be noted, has at least one carbonyl radical on the middle ring of the group. Some specific members of the indanthrene series, such as indanthrone, have two such carbonyl radicals attached to the middle ring. Others, such as flavanthrene, contain the single essential carbonyl radical, the tricyclic group being linked to a second such group by means of nitrogen linkages, or (as in the case of pyranthrone) through unsaturated hydrocarbon linkages. Thus, the two tricyclic nuclei may be linked by two  $-N=$  groups (as in flavanthrene); by two  $-NH-$  groups (as in indanthrene blue); by two  $=CH-$  groups (as in pyranthrone); or by intervening condensed ring systems (as in violanthrone). Another characteristic of the indanthrene dyes is that nitrogen is not a nuclear element present in the rings making up the essential tricyclic nuclei.

The lubricating oil chosen to form the greases of invention may be widely varied. The oil chosen to prepare the grease composition should be capable of performing the lubricating function if it could be used as a liquid. Mineral lubricating oils having a viscosity within the range of from about 35 to about 200 SUS at 210° F. may be used for most applications. The mineral oil may be of a paraffinic or of a naphthenic nature depending upon the crude source, and any of the various distillates refined by the various refinery techniques are operable.

Synthetic lubricating oils may also be utilized in preparing the lubricating greases of this invention. Synthetic lubricating oils having a viscosity within the range stated above are operable. These oils include esters of mono-basic acids, such as the  $C_8$  Oxo alcohol ester of  $C_8$  Oxo acid, esters of  $C_{13}$  Oxo alcohol and octanoic acid, etc.; esters of dibasic acids, such as di-2-ethylhexyl sebacate, di-nonyl-adipate, etc., esters of glycols, e.g., the  $C_{13}$  Oxo acid diester of tetraethylene glycol, etc., complex esters, such as the complex ester formed by reacting one mol of sebacic acid with two mols of tetraethylene glycol and two mols of 2-ethyl hexanoic acid; other types include complex esters formed by reacting one mol of tetraethylene glycol with two mols of sebacic acid and two mols of 2-ethyl hexanol, complex esters formed by reacting together one mol of azelaic acid, one mol of tetraethylene glycol, one mol of  $C_8$  Oxo acid, and the like. A recently developed class, namely diaryl dialkyl silanes (e.g., diphenyl didodecyl silane) may be employed. Esters of phosphoric acid may be used, such as the ester formed by contacting three mols of the monomethyl ether of ethylene glycol with one mol of phosphorus oxychloride. Halocarbon oils, such the polymers of chlorotrifluoroethylene may be employed, as well as alkyl silicon compounds, such as methyl polysiloxanes, ethyl polysiloxanes, methyl-phenyl polysiloxanes, ethyl-phenyl polysiloxanes, chlorophenyl silicones, and the like. Sulfite esters, such as those formed by reacting one mol of sulfur oxychloride with two mols of the methyl ether of ethylene glycol and the like also are useful, as are carbonates such as those formed by reacting  $C_8$  Oxo alcohol with ethyl carbonate to form a half ester and reacting this half ester with tetraethylene glycol, mercaptals such as those formed by reacting 2-ethylhexyl mercaptan with formaldehyde, formals such as those formed by reacting  $C_{13}$  Oxo alcohol with formaldehyde, polyglycols, such as those formed by condensing butyl alcohol with up to fifty units of propylene oxide, or mixtures of any of the above synthetic oils in an proportions.

A recent development in the high temperature lubricating field and in the allied field of lubrication under conditions of ionizing radiation comprises the use of polyphenyl ethers as lubricants or as lubricant components.

5 The maximum stability obtained if the polyphenyl ethers are unsubstituted but highly stable lubricants are also prepared when alpha-cumyl or tertiary-butyl substituents are employed. While ortho, meta or para linkages between phenyl radicals may be utilized, it is preferred that at 10 least 25% of the ether linkages be in the meta position relative to each other. As the meta linkage proportion increases, the pour point of the resulting lubricating oils decreases. It is possible to have, therefore, polyphenyl ethers which are all meta linked but which may instead 15 comprise meta linkages with varying proportions of ortho or para linkages. It is preferred that the polyphenyl ether contain from 3 to 6 phenyl radicals per molecule on the average. The combination of the subject class of thickeners with such lubricants has been found to constitute an outstandingly stable lubricating grease either under conditions of temperatures in excess of 350° F. or under conditions of ionizing radiation.

It will be understood that the addition of the amines to the subject class of greases may be utilized for the purpose of increasing the consistency of the grease on the one hand or for decreasing the major thickener requirements such as dye for a given grease consistency on the other hand. The following examples illustrate the unexpected increase in consistency of an indanthrene blue (indanthrone) grease, 28% by weight of the grease being indanthrone, the balance of the grease being a residual petroleum lubricating oil, namely, a bright stock.

| 5  | Additive                         | Percent w. | Change in W 60 Pen. <sup>1</sup> caused by amine addition | Equiv. Added per 100 g. grease | Change in W 60 Pen. <sup>1</sup> per equiv./100 g. grease |
|----|----------------------------------|------------|-----------------------------------------------------------|--------------------------------|-----------------------------------------------------------|
| 40 | Diphenylamine.....               | 4          | -37                                                       | 0.024                          | -1,540                                                    |
|    | Dinaphthylamine.....             | 3          | -16                                                       | 0.011                          | -1,460                                                    |
|    | Phenyl-beta-naphthyl-amine.....  | 4          | -37                                                       | 0.018                          | -2,050                                                    |
|    | Phenyl-alpha-naphthyl-amine..... | 4          | -40                                                       | 0.018                          | -2,220                                                    |
| 45 | Phenyl-alpha-naphthyl-amine..... | 7.5        | -71                                                       | 0.034                          | -2,080                                                    |
|    | Phenyl-alpha-naphthyl-amine..... | 15         | -86                                                       | 0.068                          | -1,260                                                    |

<sup>1</sup> Worked 60 strokes penetration, measured with  $\frac{1}{2}$  scale cone in a size "0" crucible.

50

According to the data given above, it will be seen that a variety of amines substantially increase the consistency of the grease when utilized in proportions between 3 and 15% based on the original grease formulation.

55 I claim as my invention:

1. A grease composition comprising a major amount of bright stock mineral lubricating oil gelled to a grease consistency with a combination of 5-35% by weight of indanthrone and 2.5-20% by weight of a diarylamine having the general configuration



wherein each Ar is an aromatic hydrocarbon radical of the group consisting of phenyl, naphthyl, alkylated phenyl and alkylated naphthyl radicals.

2. A grease composition comprising a major amount of bright stock mineral lubricating oil gelled to a grease consistency with a combination of 5-35% by weight of indanthrone and 2.5-20% by weight of a phenyl naphthyl-amine, the amount of said amine being sufficient to substantially increase the consistency of the grease.

3. A grease composition comprising a major amount of bright stock mineral lubricating oil gelled to a grease consistency with a combination of 5-35% by weight of indanthrone and 2.5-20% by weight of a dinaphthylamine,

75

the amount of said amine being sufficient to substantially increase the consistency of the grease.

4. A grease composition comprising a major amount of a lubricating oil gelled to a grease consistency with a combination of 5-30% by weight of an indanthrene compound and 1.5-20% by weight of a diarylamine having the general configuration



wherein each Ar is an aromatic hydrocarbon radical of the group consisting of phenyl, naphthyl, alkylated phenyl and alkylated naphthyl radicals.

5. A grease composition according to claim 4 wherein the lubricating oil is a polyphenyl ether.

References Cited in the file of this patent

UNITED STATES PATENTS

|    |           |                        |               |
|----|-----------|------------------------|---------------|
| 5  | 2,351,384 | Woods et al. -----     | June 13, 1944 |
|    | 2,403,104 | Lien -----             | July 2, 1946  |
|    | 2,663,690 | Eckert -----           | Dec. 22, 1953 |
|    | 2,848,417 | Armstrong et al. ----- | Aug. 19, 1958 |
| 10 | 2,851,418 | Lyons et al. -----     | Sept. 9, 1958 |
|    | 2,892,776 | Lyons et al. -----     | June 30, 1959 |
|    | 2,908,644 | Odell et al. -----     | Oct. 13, 1959 |
|    | 2,946,750 | Odell et al. -----     | July 26, 1960 |